

G. E. Sellers.

## *Disintegrating Process.*

Nº 40,217.

Patented Oct. 6, 1863.



Fig. 1.



Fig: 2.



Fig. 3.

Witnesses:

W.H. Townsend  
W. Maryland Avenue

*Inventor:*

Geo. E. Goldsborough

# UNITED STATES PATENT OFFICE.

GEORGE ESCOL SELLERS, OF HARDIN COUNTY, ILLINOIS, ASSIGNOR TO  
HIMSELF AND PHILIP M. PRICE.

## IMPROVEMENT IN PREPARING WOODY FIBER FOR PAPER-STOCK.

Specification forming part of Letters Patent No. 10,217, dated October 6, 1863.

*To all whom it may concern:*

Be it known that I, GEORGE ESCOL SELLERS, of Hardin county, in the State of Illinois, have invented a new and Improved Process of Disintegrating Woody Fibers for Paper-Stock; and I do hereby declare that the following is a full and exact description thereof.

The object of my invention is to separate or disintegrate woody fibers for paper-stock by a mechanical process in a cheaper and more thorough manner than has heretofore been done.

The nature of my invention consists in crushing endwise, or nearly so, the fibers of the wood or other material used, and then cutting off the crushed portion; or, what is essentially the same thing, cutting the fiber in mass into short lengths, and by an end-crushing pressure applied thereto producing separation.

In order to render the process clear to the practical mechanic, and to enable him to put it into operation, I will describe some of the many devices applicable to the process, referring to the annexed drawings, making part of this specification, in which—

Figure 1 represents a plan, part in section, of a machine for crushing and then cutting off the crushed portions of the fiber. Fig. 2 represents, also part in section, a plan of a machine in which the cutting off is done first and the crushing afterward. Fig. 3 shows the nature of the crushing above alluded to.

Similar letters on each refer to similar parts.

In Fig. 1 a log of wood, A, is represented as cut to fit into the metal box B. The box B is firmly bolted to suitable foundations, and is provided with a screw, C, and follower D, at the back end of the log, to enable it to be fed up to the crushing and cutting machine. In front of the box B is a vibrating arm, E, whose fulcrum at F is also firmly secured to the foundation. The arm E is made to carry a roller, G, and back of it a hinged knife or cutter, H. The knife H is held up against the front of the log-box B by a spring, and the end of the log-box is curved to the arc described by the arm E. At I the attachment can be made to any machine capable of imparting a reciprocating movement to the arm E, the length of stroke being limited to passing both roller and knife over the face of the

wood, and not beyond the curved or guide end of the box, so that the knife shall never fall behind the box, and thus be broken.

To use a machine of this form of construction, it is only necessary to fill the box B with a solid log of wood or pieces of wood, and to feed them up to the knife and roller by means of the screw C at each stroke of the vibrating arm; then, in making the forward stroke, the roller running in advance of the cutting-blade crushes in the woody fiber, which is then sheared off by the knife H, and on the back-stroke, the feed having been given to the wood, the knife will ride over the end of the wood and the roller will crush the fiber, and in the next forward stroke, an additional feed having been given to the wood, will again crush it in advance of the knife, thus twice passing over the end of the wood before the fibers are cut to length. In this form of machine the fibers are crushed before being cut off. The action of the roller in twice passing over the end of the wood has a tendency, in addition to the direct-crushing pressure, to bend the fibers in the direction the roller is passing, and in soft woods—such as the cotton-wood, (*Populus angulata*)—greatly aids in separating them; but when the wood is hard and the strain on the machine would be too great, the cutting may be done first, as in Fig. 2, and the shaving of wood may be guided between two rollers, G and G', which will effect the crushing endwise in as effectual a manner as in the first instance, the amount of crushing being regulated by the screws J and J', which adjust the distance apart of the rollers G and G', and in this case the knife may be a stationary one, as it does not have to yield back as it repasses the end of the wood, the feed being made just before the knife begins to cut. In order the better to preserve the wood thus cut in a perfect sheet, an end plate, K, may be placed for the knife to cut up against or behind it, this plate serving to force the wood which has been cut off into the guides L and L'. It is evident that the wood thus forced into the rolls will of itself cause their rotation; but if it is deemed advisable they may be made to rotate by any of the well-known mechanical devices.

I have described these two general methods of working my process, in order to show that

it is not confined to any one special device, but may be accomplished in various ways; and I would still further suggest that the wood might be sawed across the grain into thin sheets, and then passed between any ordinary plain rollers to crush it endwise, or could be crushed by hammering or steady pressure between plain plates. After crushing and cutting, or cutting and crushing, I pass the fiber through a common thrashing-machine or wool-picker, more perfectly to separate the fibers one from another.

I am aware that there is no novelty in cutting or chopping into short lengths woody fiber in preparation for paper-stock; but all the processes heretofore used to reduce the woods fine enough to be economically operated on by the chemicals used to remove the gum resins, and other substances that cement the fibers together, break up, cut, or destroy the uniformity in the length of the fibers in a much larger proportion than by my process, which forces or tears the fibers apart, reducing them to a cottony mass easily separated, and in such a condition as to be operated on by the smallest amount of chemicals. The strength of paper depends much on the length of the fiber, and its quality on their uniformity; hence the importance of separating woody fiber in the most perfect manner previous to freeing it from its gums, bleaching and pulping it. Whenever practicable, woody fibers should be separated when in a green state, or as soon as possible after the timber

is felled. The separation is most perfectly made when the timber is cut in full leaf and well filled with sap, and the gum resins are removed with less cost and labor than when the sap is not in the wood. When the wood becomes partially seasoned or dried, it must be softened by soaking or steaming, care being taken not to overheat it, as high temperatures drive the gums into the fibers themselves, and they then require more severe chemical treatment to remove them and to bleach the stock. The fibers of the hemlock, spruce, (*Abies canadensis*), and many of the species *coniferae* are with facility separated by my process, producing long and strong fiber well adapted for paper-stock, but abounding in gum resins. The bass-wood, (*Tilia americana*), poplar or tulip tree, (*Syriodendron tulipifera*), and the two varieties of cotton-wood, (*Populus canadensis* and *angulata*), are also easily operated on and produce a good fiber for paper-stock.

Having thus described my invention, as to its object, nature, and theory of operation, what I claim as new, and desire to secure by Letters Patent, is—

The separating or disintegrating of woody fiber for paper-making by pressure in the line, or nearly so, of the fiber, substantially in the manner above described.

GEO. ESCOL SELLERS.

Witnesses:

JOHN F. LEDBETTER,  
LOUIS S. DENNIS.